

## UNITED STATES PATENT OFFICE

1,973,998

## SIZING ARTIFICIAL SILK

Paul Schlack, Berlin-Lichtenberg, and Ernst Sauter, Berlin-Karlsborst, Germany, assignors to Aceta G. m. b. H., Berlin-Lichtenberg, Germany, a corporation of Germany

No Drawing. Application January 17, 1931, Serial No. 509,537. In Germany January 21, 1930

16 Claims. (Cl. 134—18)

Our invention relates to an improved sizing preparation for artificial fibers and more especially for such fibers as are made from cellulose acetate, which facilitates subsequent operations, 5 said sizing materials being of the type employing a drying oil.

One of its objects is to provide sizing agents comprising as a main part drying oils said sizing agents yielding elastic coatings so that the sized 10 fiber remains soft and does not break when bent. It may be applied without injuring the fiber and can be easily and economically removed without damage to the fiber.

Preparations meeting all of the requirements, 15 are obtainable according to our invention by adding to the drying oils another oil of high viscosity, said second oil being a non-drying oil or an incompletely drying oil.

As drying oils being the chief ingredient in our 20 size preparations, we enumerate, for instance, the following:— linseed oil, soy bean oil, perilla oil, water oil, rape oil, or cotton oil, preferably purified from their slimy impurities.

As a softening oil preventing the sizing film from 25 breaking, we may use chemically altered natural or artificial oils having at 100° C. a viscosity of more than 10 or preferably more than 20° measured with the Engler viscosimeter and an iodine number not higher than 60, preferably between 30 40 and 50. Representatives of these groups of practically non-drying oils are the following:— highly oxidized unsaturated oils or fats such as, for instance, blown rape oil, blown cotton oil, blown soy bean oil, etholide glycerides, or free 35 etholides such as formed, for instance, by heating a higher hydroxy fatty acid, whereat an esterification of a number of hydroxy fatty acid molecules occurs (cf. K. H. Bauer, Fette und Oele, 1928, printed by Parey, Berlin, pages 80, 40 108 and 386). Preferably blown half-drying oils of commerce, for instance, blown rape oil, may be used. The quantity of softening oil, we add, amounts to 5-30% calculated on the quantity of the drying oil.

45 Our new preparations may be used together with drying accelerators such as cobalt acetate, cobalt oleate or cobalt resinate or with one of the known manganese or lead dryers the quantity of which depends on the drying period desired. 50 By suitably choosing the amount of the drying accelerator to be added the removal of the sizing agent may be improved. They may be used either together with a solvent, for instance, an aromatic or aliphatic hydrocarbon, or in 55 form of aqueous emulsions prepared in the known

manner with aid of a soap or an emulsifier, for instance, Turkey red oil, whereat the emulsification of the drying oils is facilitated by the presence of the blown oils or the etholides. In certain cases it is advisable to add oil-soluble soaps made from water soluble amines, preferably amine soaps, for instance, triethanol amine, which soaps prevent a too rapid drying of the sizing.

A sizing or coating of these preparations applied to the fiber adds to its strength, makes the individual fibers of a thread glue together and prevents opening in the loom or elsewhere; it adds to the elasticity of the thread, prevents it from being charged with static electricity and the thread follows easily all the movements necessary when traveling in contact with parts of the machine by which it is made up into a fabric. The subsequent separation of the sizing from the fiber presents no difficulty and can be carried out without injuring the fiber. For the removal of the sizing there may be used the known agents, for instance, a soap solution containing a perboric acid salt. Contrary to the known sizing preparations made with drying oils, our sizing materials effect a certain adhesion of the individual fibers before drying of the oils without sticking of the threads. This adhesion of the individual fibers is desired, for instance, in the case of only slightly twisted artificial silk or if the sized material is subjected before drying to a textile operation, for instance, to twisting, which may occur, if the sizing agent is applied to the running thread in the dry-spinning process.

Our invention is illustrated by the following examples:—

Example 1—Preparation for sizing acetate silk in skeins

80 parts of purified linseed oil are mixed with 19 parts of blown rape oil (viscosity  $E_{100^{\circ}}=30$ , iodine number: 46), 0.6 parts of lead resinate, 0.4 parts of manganese resinate and 400 parts of high-boiling benzine. The skeins treated with this preparation are centrifuged and hung until the sizing film has dried throughout.

Example 2—Preparation for sizing the linearly running thread spun on the dry spinning machine

A sizing preparation useful for the process as set forth, may consist of 85 parts of purified linseed oil, 15 parts of blown rape oil (viscosity  $E_{100^{\circ}}=40$ , iodine number: 43), 0.2 parts of a mixture of lead and manganese resinate mixed in the ratio 2:1, and 100 parts of toluene. The solution is applied

on the running threads through capillary nozzles, the threads are twisted and hung in form of skeins until the sizing film has dried.

*Example 3.*—The sizing preparation is composed according to the following formula:—15 parts of etholide glyceride made from ricinoleic acid (viscosity  $E_{100}^{\circ}$  = 16, iodine number: 88), 0.5 parts of a mixture of 3 parts of lead naphthenate and 1 part of manganese naphthenate dissolved in 5 parts of linoleic acid, and 400 parts of high-boiling benzene or solvent naphtha. This solution is useful in sizing skeins of artificial silk.

What we claim is:—

1. A sizing preparation comprising a drying oil and a practically non-drying oil having a viscosity of  $E_{100}^{\circ}$  c. higher than 10.

2. A sizing preparation comprising a drying oil and a blown half-drying oil having a viscosity of  $E_{100}^{\circ}$  c. higher than 10 and an iodine number below 60.

3. A sizing preparation comprising a drying oil, a blown half-drying oil having a viscosity of  $E_{100}^{\circ}$  c. higher than 10 and an iodine number below 60, and a small quantity of a drying accelerator.

4. A sizing preparation comprising 80 parts by weight of purified linseed oil and 19 parts by weight of blown rape oil having a viscosity of  $E_{100}^{\circ}$  c.=30 and an iodine number of 46, 0.6 parts

30 by weight of lead resinate, 0.4 parts by weight of manganese resinate and 400 parts by weight of high-boiling benzene.

5. A sizing preparation comprising 85 parts by weight of purified linseed oil, 15 parts by weight of blown rape oil having a viscosity of  $E_{100}^{\circ}$  c.=40 and an iodine number of 43, 0.2 parts by weight of a mixture of lead and manganese resinate mixed in the ratio 2:1, and 100 parts by weight of toluene.

40 6. A sizing preparation comprising 15 parts by weight of etholide glyceride made from ricinoleic acid having a viscosity of  $E_{100}^{\circ}$  c.=16 and an iodine number of 83, 0.5 parts by weight of a mixture of 3 parts by weight of lead naphthenate and 1 part by weight of manganese naphthenate dissolved in 5 parts by weight of linoleic acid, and 400 parts by weight of high-boiling benzene.

50 7. A sizing preparation comprising a drying oil and an oil of the group consisting of a blown half-drying oil having a viscosity of  $E_{100}^{\circ}$  c. higher than 10 and an iodine number below 60, a free etholide and an etholide glyceride.

8. Artificial silk threads consisting of hydrated cellulose or a cellulose derivative coated with a sizing preparation comprising a drying oil and an oil of the group consisting of a blown half-drying oil having a viscosity of  $E_{100}^{\circ}$  c. higher than 10 and an iodine number below 60, a free etholide and an etholide glyceride.

60 9. Artificial silk threads consisting of hydrated

cellulose or a cellulose derivative coated with a sizing preparation comprising a drying oil and a blown half-drying oil having a viscosity of  $E_{100}^{\circ}$  c. higher than 10 and an iodine number below 60.

10. Artificial silk threads consisting of hydrated cellulose or a cellulose derivative coated with a sizing preparation comprising a drying oil, a blown half-drying oil having a viscosity of  $E_{100}^{\circ}$  c. higher than 10 and an iodine number below to 60, and a small quantity of a drying accelerator.

11. Artificial silk threads consisting of hydrated cellulose or a cellulose derivative coated with a sizing preparation comprising 80 parts by weight of purified linseed oil and 19 parts by weight of blown rape oil having a viscosity of  $E_{100}^{\circ}$  c.=30 and an iodine number of 46, 0.6 parts by weight of lead resinate, 0.4 parts by weight of manganese resinate and 400 parts by weight of high-boiling benzene.

12. Artificial silk threads consisting of hydrated cellulose or a cellulose derivative coated with a sizing preparation comprising 85 parts by weight of purified linseed oil, 15 parts by weight of blown rape oil having a viscosity of  $E_{100}^{\circ}$  c.=40 and an iodine number of 43, 0.2 parts by weight of a mixture of lead and manganese resinate mixed in the ratio 2:1, and 100 parts by weight of toluene.

13. Artificial silk threads consisting of hydrated cellulose or a cellulose derivative coated with a sizing preparation comprising 15 parts by weight of etholide glyceride made from ricinoleic acid having a viscosity of  $E_{100}^{\circ}$  c.=16 and an iodine number of 88, 0.5 parts by weight of a mixture of 3 parts by weight of lead naphthenate and 1 part by weight of manganese naphthenate dissolved in 5 parts by weight of linoleic acid, and 400 parts by weight of high-boiling benzene.

14. A sizing preparation comprising a drying oil and an oil of the group consisting of a blown half-drying oil having a viscosity of  $E_{100}^{\circ}$  c. higher than 10 and an iodine number below 60, a free etholide and an etholide glyceride, and a small quantity of a drying accelerator.

15. Artificial silk threads consisting of hydrated cellulose or a cellulose derivative coated with a sizing preparation comprising a drying oil and a practically non-drying oil having a viscosity of  $E_{100}^{\circ}$  c. higher than 10.

16. Artificial silk threads consisting of hydrated cellulose or a cellulose derivative coated with a sizing preparation comprising a drying oil and an oil of the group consisting of a blown half-drying oil having a viscosity of  $E_{100}^{\circ}$  c. higher than 10 and an iodine number below 60, a free etholide and an etholide glyceride, and a small quantity of a drying accelerator.

PAUL SCHLACK.  
ERNST SAUTER.

135

65

140

70

145

75

150